

June 4, 1963

E. J. RIPLING

3,092,470

**E. S. RIFLING** **3,032**  
PREPARATION OF SHEET STOCK HAVING LONGITUDINAL EXTERNAL

## WEAKENINGS THEREIN AND PRODUCT THEREOF

Filed July 29, 1959

3 Sheets-Sheet 1



INVENTOR

EDWARD J. RIPLING

BY *Mason, Porter, Dillon & Stewart,*  
ATTORNEYS

June 4, 1963

E. J. RIPLING

3,092,470

PREPARATION OF SHEET STOCK HAVING LONGITUDINAL EXTERNAL  
WEAKENINGS THEREIN AND PRODUCT THEREOF

Filed July 29, 1959

3 Sheets-Sheet 2

FIG. 5



FIG. 6



FIG. 7



INVENTOR

EDWARD J. RIPLING

BY *Mason, Porter, Dillon & Stewart,*

ATTORNEYS

June 4, 1963

E. J. RIPLING

3,092,470

PREPARATION OF SHEET STOCK HAVING LONGITUDINAL EXTERNAL  
WEAKENINGS THEREIN AND PRODUCT THEREOF

Filed July 29, 1959

3 Sheets-Sheet 3

FIG. 9



FIG. 10



INVENTOR

EDWARD J. RIPLING

BY *Mason, Porter, Diller, & Stewart,*  
ATTORNEYS

# United States Patent Office

3,092,470

Patented June 4, 1963

1

3,092,470

## PREPARATION OF SHEET STOCK HAVING LONGITUDINAL EXTERNAL WEAKENINGS THEREIN AND PRODUCT THEREOF

Edward J. Ripling, Flossmoor, Ill., assignor to Continental Can Company, Inc., New York, N.Y., a corporation of New York

Filed July 29, 1959, Ser. No. 830,339  
16 Claims. (Cl. 29—187)

This invention relates to the preparation of sheet stock having longitudinal external weakenings therein, and concerns particularly the preparation of a rolled stock having internal discontinuities and external weakenings accurately located relative to one another.

It is known to produce metallic sheet and strip stock by rolling, and to subdivide it subsequent to rolling by slitting or a like severing operation. It is also known to produce sheet material having internal discontinuities by a rolling operation which reduces the billet thickness and extends its length. The billet is provided with one or more internal channels prior to final rolling, usually when the billet is first prepared, with a content of an anti-welding or resist material which is likewise reduced in thickness and extended during the rolling, so that the resist serves to prevent welding at the discontinuity regions; wherewith the rolled strip produced is of laminate structure, comprising surface laminations of the billet metal separated by the residues of the resist material at the discontinuity regions, and with these laminations joined by integrating metal along the longitudinal edges and along longitudinal strips or spacers between adjacent discontinuity regions. When two or more such discontinuities are present, the strip is called "multi-wide" because it can be slit through the integrating metal or spacers and thus severed into a number of narrower strips each of which has a discontinuity therein and each of which has integrating metal connections at its edges.

The word "billet" is employed herein to designate a body produced as a cast ingot, or by a body produced by bonding slabs through rolling or brazing. Correspondingly, the word "lamination" is employed herein to designate a layer of the billet material which provides a surface of the strip and is separated from a cognate lamination, toward the end of the rolling schedule, by the layer of residual anti-welding material.

The rolling operation, for converting the billet to the strip, usually results in a strip having "camber" with one or both edges departing from straight lines; and then, when one or more internal discontinuities are present, the edges thereof are no longer straight and in the longitudinal direction of the rolling. Likewise, a widening of the stock occurs, and this widening is not uniform throughout the thickness and frequently the strip does not have parallel straight edges. Further, when an internal discontinuity is present, in practice the reduction of the original thickness of resist material may bring this to a thickness of 0.001 inch or less; and it is then difficult to discover the exact position occupied by a discontinuity in the rolled strip. When a strip is rolled "multiwide," with or without internal discontinuities, it is frequently desired to be able to trim it to have parallel edges whether straight or not; and to be able to subdivide it into narrower strips with edges which are essentially parallel in each strip.

One use for such strips is in the making of tubular bodies, by employing mechanical means or fluid pressure to cause the laminations to bend away from one another. Wherewith the integrating metal connections at the edges of a single-wide strip remain as externally projecting fins having a thickness about twice that of the laminations, in

2

this illustrative example. The slitting of the multi-wide strip for producing the single-wide strips must be at accurately located longitudinal lines, because an intrusion of the separating slit into or too close to a discontinuity will cause cracking and leakage of the tube produced. It is feasible to have the integrating metal relatively wide, to permit the slitting along the same at lines safely distant from adjacent discontinuity regions, and then to trim away excess after the tube has been opened; but this represents an uneconomic loss of the metal thus trimmed away. That is, these integrating regions should be made as narrow as possible.

It has been found that the separation of a multi-wide strip into narrower single-wide strips can be effected by providing in the wide strip longitudinal lines of weakening; and that such weakenings can be produced at accurately preselected regions by preliminary treatment of the billet before its rolling is completed. This procedure is likewise effective with rolled strip stock, in providing weakenings by which irregular edge portions of the strip can be detached, to provide edges which are essentially straight for strip lengths of sheet to be cut therefrom and thus provide accurate guide edges from which such cuts can be made.

One of the objects of this invention is the process of preparing a billet having longitudinal surface irregularities which become accurately positioned external weakenings in the wide strip rolled from the billet and permit longitudinal severance into narrower strips having their edges accurately located relative to one another.

Another object is the process of preparing a billet by providing an open longitudinal groove on its surface, with a weld-preventing or resist material therein, and then rolling to reduce the billet to the desired final thickness and therewith closed the groove wherewith the resist material maintains the weakening effect introduced by the said groove.

A further object is the process of preparing a billet by providing longitudinal surface grooves at different spacings from its center, and then rolling to reduce the billet to the desired final thickness and therewith provoking a differential lateral spreading across the width as the strip is formed, wherewith the differential spreading compensates for and coordinates with the differential original spacing so that the groove residues in the final strip are spaced at positions determined in the billet before rolling.

A further object is the production of a multiwide strip having a plurality of internal discontinuities spaced from one another across the width of the strip by integrating metal connecting the surface laminations at the edges of the discontinuity regions, and with external weakenings accurately located at the integrating metal regions and spaced from the edges of adjacent discontinuity regions.

With these and other objects in view, as will appear in the course of the following description and claims, illustrative practices are shown in the accompanying drawings, in which:

FIGURE 1 is an end view of an ingot prepared according to this invention;

FIGURE 2 is an end view on a larger scale, of part of a multi-wide strip prepared from the ingot of FIGURE 1;

FIGURE 3 is an end view of a modified form of billet; FIGURE 4 is an end view on a larger scale of a part of a multi-wide strip prepared from the billet of FIGURE 3;

FIGURE 5 is a perspective view of two slabs for forming a billet;

FIGURE 6 is a diagrammatic view, at greatly enlarged scale, of a billet groove with resist material therein, and

showing in dotted lines the condition after a partial rolling;

FIGURE 7 is a diagrammatic view, corresponding to FIGURE 6 but showing the weakening present after rolling;

FIGURE 8 is a diagrammatic view illustrating a manner of separating the strip;

FIGURE 9 is a perspective view showing removal of an edge portion from a strip;

FIGURE 10 is a conventionalized showing of an apparatus for flexing and notch breaking a section of the strip of FIGURE 9;

FIGURE 11 is a perspective view of a conventionalized apparatus for longitudinally ripping the strip of FIGURE 9.

An ingot may be prepared by casting a metal, e.g., steel or aluminum in a mold, to provide the body B in FIG. 1. Incidental to the casting, or by subsequent operation thereafter, longitudinal channels 10 can be provided and filled with an anti-weld or resist material appropriate to the metal, the temperature to which it is subjected during the rolling schedule, and the purpose for which it is to be used. Finely powdered aluminum oxide, titanium oxide, silicon oxide, talc, graphite, and like refractories are useful with hot rolling schedules; noting that graphite should not be employed if its presence will damage the product, e.g., by electrochemical effects or by the creation of undesirable carbide concentrations. Such an ingot may be made of a transverse dimension accepted by the rolls to be employed; and therewith may have a number of the core channels 10 spaced across its width: more than three being indicated in FIGURE 1, noting that each core channel is to provide an internal discontinuity in the multi-wide final strip. The metal above and below the core channels in FIGURE 1 is integrated by metal connections 11, 12 at the longitudinal edges and between adjacent channels.

According to this invention, the ingot body B of FIGURE 1 also has longitudinal grooves 14 provided therein, being present opposite the intermediate integrating connections 12. In FIGURE 1, such are shown at both top and bottom faces of the ingot; but it will be understood that employment of only one such groove opposite each connection 12 is comprised in the invention. Such grooves may be formed by mold wall projections, or can be later cut or impressed mechanically.

Upon rolling the ingot of FIGURE 1, the grooves 14 are closed to give essentially smooth surfaces in the final multi-wide strip, as shown in FIGURE 2, where the metal laminae 15, 16 are separated by the residues 17 of the cores, and are connected at the edges of such residues by the integrating residues 18 of the connections 11, 12 of FIGURE 1. The grooves have been closed, but their walls begin to abut along planes essentially normal to the ingot surfaces and hence no substantial welding pressure is being exerted therebetween. It is preferred to coat one or both walls of each groove with an adherent coating 19 of resist or anti-welding material, so that the same is present when the groove becomes closed: during rolling the dimension of this resist material, in the transverse direction of the ingot, remains essentially the same, but its dimension in the direction between the rolled surfaces of the ingot is reduced essentially in proportion to the reduction of the metal stock and of the resist material in the channels.

During the course of the rolling, the over-all thickness is decreased, and therewith the ingot becomes a strip S, FIGURE 2: with an increase of width of up to 14 percent dependent upon the material and the treating and rolling schedule, and amounting to say  $\frac{1}{2}$  percent with a long schedule of low reductions and up to 14 percent with a schedule of very heavy reduction per pass: in practice a spread of 4 to 5 percent is a desirable amount for an economical rolling schedule. The ingot B tends to spread more at one or more planes between the surfaces than

at its top and bottom surfaces, noting that the friction between each roll and the surface contacted thereby act to restrict surface spreading at the surface planes X. The spreading may differ at successive planes from the surfaces toward the median or central plane: e.g., when the reduction per pass is small, the spread adjacent the surfaces is greater than that at the median plane; while with high reduction per pass, the spread at the median plane M is usually greater than at any plane between the median and surface planes. Therewith the residues 20 of the grooves tend to shift from positions at right angles to the surfaces to positions at acute angles, the angle increasing from the center of width toward the edges, as shown in FIGURE 2; but with the inner edge of each groove remaining aligned with its associated integrating metal or spacer 18. In general, if each groove has an original depth of about one-third the thickness of the ingot, each residue 20 is less than one-third of the total thickness of the strip, and two opposed grooves will be separated by a distance of about half the total thickness measured through the integrating metal. As a specific example, the ingot B of FIGURE 1 may have a thickness of  $1\frac{1}{2}$  inches, with each core channel 10 0.060 inch thick and filled with resist and having the integrating metal connections about 0.125 inch wide, and with the grooves 14 each shaped as a 45 degree V and cut 0.350 inch deep with a resist coating 19 about 0.020 inch thick; then upon rolling, the integrating connections widen during rolling to 0.130 to 0.150 inch, dependent upon the rolling schedule, when

the strip has been reduced to a total thickness of 0.025 inch comprised at the discontinuity regions of two metal laminae 15, 16 which are each 0.012 inch thick and separated by a resist residue 17 which is 0.001 inch or less thick, and having the integrating connections 18 0.025 inch thick from face to face of the strip; therewith the groove residues 20 are about 0.005 to 0.010 inch in the transverse direction of the strip and extend into the integrating metal for about 0.0025 to 0.005 inch each. It will be noted that therewith the distance between opposed groove residues is about 0.017 inch, with each residue separated by about 0.062 inch from the adjacent edges of the core residues 17.

It has been found that such grooves, FIGURE 1, with an included angle of 45 degrees, are effective, when such aligned grooves are formed in the upper and lower surfaces and to a depth of 23 percent of the billet thickness for each, or 46 percent in all. During the initial rolling passes, and with the metal being spread laterally to close the open groove volumes, the metal between the roots of a pair of such grooves is not reduced proportionately to the reduction of the metal at points intermediate two pairs of grooves. For example, a customary rolling procedure results in the residues of these grooves being each about 18 percent of the total thickness of the strip when reduced to final gauge, or 36 percent for the two. In general, the notches should originally have included angles less than 90 degrees, and more than about 20 degrees when spray coating thereof is employed: preferably the angle should be between 25 and 75 degrees, noting that the angles of successive grooves in a single billet may differ. Similarly, it is preferred to have the depth of each groove between 10 and 25 percent of the billet thickness, again noting that all grooves on a single billet need not have the same depth.

In the form of FIGURES 3 and 4, the billet B illustratively has four cores 10, two being disposed symmetrically to the longitudinal central upright plane indicated by line 25, with two cores between such plane and each longitudinal edge. Aligned with the integrating connections 12, in FIGURE 3, are the pairs of grooves 14a, 14b, 14c. In the form of FIGURE 3, the grooves 14b, 14c are tilted relative to longitudinal upright planes so that each groove has its side which is nearer the center plane 25 at a greater angle to the billet surface than the side which is farther from the center; and for each suc-

cessive groove the tilting is greater for a groove near the edge than for a groove nearer the center: the angle of tilt likewise being coordinated to the material and treatment schedule. Expressed in another way, when the rolling schedule produces a greater spread at the intermediate planes  $P$  than at the surfaces  $X$ , the bisectors of the root angles of the illustrated V cross-sections of the grooves can be at successively greater angles to the surfaces of the billet, from its center of width toward its lateral edges, as indicated by the greater angularities  $D$  of the bisector lines  $14m$  than the angularities  $C$  of the bisector lines  $14c$  in FIGURE 3, with the bisectors of each pair of grooves in the illustrative form intersecting one another at the median plane  $M$  and at a point closer to the center plane  $25$  than the roots of the V sections from this center plane. Illustratively, the tilt angles  $C$  may be 2 to 4 degrees and the tilt angles  $D$  6 to 12 degrees, with 45 degree grooves in an 8 inch billet.

Furthermore, if the rolling schedule is such that the spreading at the median plane  $M$  is significantly greater than that at intermediate planes  $P$ , a further compensating effect can be provided by varying the locations of the groove roots relative to the adjacent cores  $10$ . Thus, in FIGURE 3, the longitudinal upright central geometric plane of line  $25$  intersects the median plane  $M$  at equal distances from the adjacent cores  $10$ , and passes through the roots of the central grooves  $14a$ : that is, if the spacing between adjacent edges of the cores is 0.125 inch, the plane  $25$  is 0.0625 inch from each. Illustratively, the several core spacings are 0.125 inch, and the longitudinal upright geometric planes  $25k, 25m$  intersect the median plane  $M$  at distances of 0.0625 inch from adjacent cores  $10$ . The longitudinal upright geometric planes  $25k, 25m$  through the groove roots of the respective pairs of grooves  $14b, 14c$  are spaced laterally outward from the adjacent planes  $26k, 26m$ . Thus a plane  $25k$  may be 0.020 inches from its adjacent plane  $26k$ ; and a plane  $25m$  0.040 inch from its adjacent plane  $26m$ . These values are proper for a rolling schedule by which the total lateral spread, or gain of width, is about 4 percent at the median plane  $M$ . It will be understood that the expression "geometric" is employed to designate a plane or surface of reference, which need not be a superfcies or boundary face of a part.

Upon rolling the billet  $B$  of FIGURE 3, the grooves are closed by the transverse displacement of metal of their walls, and the resist material is therewith abutted at both sides by metal which is held against welding by this resist material. As the rolling progresses, the residues are at right angles to the rolled surfaces of the strip upon completion of the rolling. Since the widening of the billet is essentially zero at the surfaces  $X$  and is greater between these surfaces, in a fashion symmetrical relative to the median plane  $M$ , the two residues  $20a$  (FIGURE 7) of a pair therewith lie in an upright longitudinal geometric plane  $35$  and by the greater spreading at the median plane  $M$  than at the intermediate planes  $P$  for the specified schedule, the integrating metal connections  $12$  move laterally outward relative to the groove residues, so that the roots of residues  $20a$  of the pairs of grooves lie in respective upright geometric surfaces which pass through the integrating metal connections  $18$  of the strip at uniform and predetermined distances from the adjacent edges of resist residues  $17$ , e.g., exactly midway between two such residues.

The course of the early flow of metal during rolling, to close the grooves of a body  $B$ , FIGURES 1 and 3, is shown in FIGURE 6, in which a part of the body  $B$  has a groove  $20m$  therein, with a coating of resist material  $19$  on one wall  $27$  thereof, while the other wall  $28$  is illustratively bare. During the initial part of the rolling, e.g., hot rolling, the surface  $29$  is depressed to a level  $29a$  by a reduction of  $d_1$ ; wherewith the metal flows laterally to fill the groove, with the metal of wall  $27$  carrying the resist material with it and thus bringing it to abutment by the metal flowing from the wall  $28$ . This phase of roll-

ing results in a smooth surface formed by metal and resist material: it being noted that surface metal of the body between the grooves is being extended longitudinally by rolling essentially in proportion to the reduction in height from surface level  $29$  to surface level  $29a$  as a fraction of the thickness of the billet; whereas the reduction  $d_2$  below the original root of the groove is less than the reduction  $d_1$ . Therewith, while the distance from the root of a groove to an adjacent core  $10$  may be less in the original ingot than the distance between the roots of the grooves of a pair, the reduction to strip thickness leaves the lateral core spacing essentially unchanged, e.g., 0.125 inch, while the total strip thickness of 0.025 inch now has groove residue weakenings extending from its surfaces and spaced 0.008 inch apart, which is less than the distance from either weakening to the adjacent core residue.

The effect of the external longitudinal weakening is illustrated in FIGURE 7, in which the body of strip  $S$  has groove residues  $20a$  extending from its surface for about one-third of the thickness each. When tensile forces are applied, the resulting pattern (indicated by the dotted lines) will contain a great concentration of stresses at the upright plane  $35$  of the residues  $20a$  rather than in the rest of the integrating metal  $18$  and in the laminated regions above and below the resist residues  $17$ . A like concentration occurs when bending forces are exerted, or shearing forces exerted along the plane of the residues  $20a$ . Therewith the metal at such plane yields, and breakage thereat can be accomplished without significant yielding at other places.

The billet  $B$  may be formed with cores in other ways, including those taught in the Valyi et al. United States Patent No. 2,375,334, and provided with external longitudinal grooves. Thus, in FIGURE 5 are shown two like slabs  $30, 31$  which may be formed by extruding aluminum which provide longitudinal ribs  $32$  at one surface and longitudinal grooves  $33$  at the other surface and aligned with the ribs  $32$ . The ribs  $32$  define channels  $34$  which can be filled with a slurry of the resist material and baked. The exposed edge surfaces of the ribs  $32$  are cleaned of any adherent resist. The upper slab  $30$  is then inverted and placed over the lower slab  $31$  so that the ribs  $32$  abut. The assembly may be initially maintained by edge welding; and hot rolling is then employed to secure bonding between the abutting surfaces of the ribs  $32$ . Surfaces of the grooves  $33$  may be provided with resist  $19$  before or after the assembly. The assembly is then subjected to the rolling schedule, for producing a strip  $S$  as in FIGURE 2 or 4.

In FIGURES 3 and 4, the edge grooves  $14c$  and their residues  $20a$  permit the production in the final strip of a break along an upright surface  $35$  (FIGURES 8 and 9) which is parallel to the edge of the adjacent resist  $17$  and at a predetermined distance therefrom, regardless of camber of the strip or local irregularities of the strip edge. The narrow edge piece can then be broken away, and forces applied at distances measured from this guide edge. It will be noted that this break is accomplished independently of the presence of the illustrated resist residue: and that a solid sheet or strip may likewise have its edge detached, or be separated into narrower strips. Thus in FIGURE 8, the strip  $S$  has had an edge portion  $36$  thus removed; thereupon the width of the adjacent single-wide portion  $S-1$  can be closely determined, and the multi-wide strip supported at the area of the next single-wide portion  $S-2$ , as indicated by the force arrow  $37$  and this portion  $S-2$  held by a force  $38$  against its upper surface. A bending force, indicated by arrow  $39$  can then be exerted upon the upper surface of the portion  $S-1$  so that the latter bends downward toward the position shown by the dash lines, hinging about the longitudinal weakening at the plane  $40$  through the residues  $20a, 20c$  of FIGURE 7, and breaking.

Such separation of the narrow strips from one another can be accomplished in other ways. In FIGURE 9, the

strip S has the edge weakening 35 as before. A break is started at one end of the strip, and the edge portion 36 can then be torn away, noting that the severance is controlled by and follows the surface represented by the line 35 in FIGURES 7, 8 and 9, at the predetermined distance from the edge of the nearest residue 17.

The multi-wide remainder of the strip S, shown as six-wide in FIGURE 9, may now be cut transversely, e.g., at lines 41 to provide sections which can then be moved between breaker rolls 42 which act to flex and bend the section T, wherewith the material at the surfaces containing the residues 20a of FIGURE 7 are stressed beyond recovery, and breakage is produced, between the narrow strip portions V of the section T at accurately located places determined by the residues 20a. The breaker rolls 42 are positioned in upper and lower sets in FIGURE 10, with the lower tangent of the upper set of rolls located below the upper tangent of the lower set, so that the section T, shown by dotted lines in FIGURE 10, is successively flexed in opposite directions through half angles of 45 degrees or through bends of short radii established by rolls, until it separates. When the broken sections V are so narrow that they cannot contact three rollers to assume the flexing and continued movement in the apparatus, they may be controlled during passage between the rolls 42 by the belts 45, which may be relatively loose so that the panels formed by the successive narrow strips in hinging about the longitudinal weakenings can retain relative flatness without conforming to the rolls 42 in passage therebetween. With wider strips V, the belts 45 may be omitted.

The narrow strips may also be produced as an incident of coiling. In FIGURE 11, the strip S is delivered between the shafts 50, 51 of two take-up reels. The end of strip S is split along the individual lines 35 between the narrow strips S-1, S-2, S-3, S-4, S-5 and S-6 thereof; and the ends of alternate strips, illustratively strips S-1, S-3 and S-5, are connected to the upper driven shaft 50, and the ends of the other strips, illustratively strips S-2, S-4 and S-6, connected to the lower driven shaft 51. As the shafts rotate in the direction shown by the arrows, the individual strips are wound onto the shafts to form the rolls R-1, R-2, R-3, R-4, R-5 and R-6; noting that any two rolls on each shaft are spaced axially by the width of the strip being wound on the other shaft in alignment with such space, and that the peeling or shearing effect as the narrow strips are pulled along their lines of longitudinal weakness while the general area of each strip is being supported by the contact therewith of the already-wound part of that strip.

In practice, it has been found that notches of V cross-section, with the roots having angles of about 10 to 55 degrees, are satisfactory. Such a notch with an inner or root angle of 45 degrees can be coated with anti-welding material along one wall, to a thickness of 0.005 to 0.020 inch by flame spraying, by deposit and baking of a slurry of the resist material, or by powder deposit into a sharp-angled groove followed by peening the outer lips together to enclose the powder. When sharper root angles, e.g., 8 degrees, are employed, the lateral spreading of the metal to close the groove usually causes a thickened section of the resist material to form adjacent the root of the notch; grooves with inner or root angles of over 60 degrees did not close regularly but tended to become shallower; whereas angles within the stated range cause the resist material to provide a weakening of substantially constant width in the direction from side to side of the rolled strip, and often with a fairly sharp angle at its inner edge.

The lateral closure of the grooves provides smooth rolled surfaces on the multi-wide strip. For example, with a billet originally 1.50 inches thick, and having aligned pairs of notches of 45 degree V section and 0.35 inch deep, no visible indentations were present on the rolled surfaces upon reduction to 0.25 inch thick. Upon rolling

billets to an over-all thickness of 0.018 inch, the differential lateral spreading was found to vary with the billet material, its heat treatment before and during rolling, and the rolling schedule, that is, the number of passes and the reduction per pass.

It is obvious that the illustrative practices are not restrictive, and that the invention can be employed in many ways within the scope of the appended claims.

What is claimed is:

1. The method of preparing narrow strips of material each having an internal discontinuity between surface laminations, the laminations being connected at the lateral edges of the discontinuity, which comprises preparing a billet of the material with a plurality of internal longitudinal channels spaced laterally from one another and from the longitudinal edges of the billet by portions of solid metal extending from face to face of the billet, said channels containing extensible weld-preventing material, said billet having a plurality of longitudinal external grooves at a roll-engaging face thereof, each of said grooves being located opposite one of the said solid metal portions, the parts of said solid metal portions beneath the roots of said grooves being effective to maintain integrity of the billet from side to side during rolling, placing a weld-preventing material on a wall of each groove, rolling the billet longitudinally whereby to cause lateral closure of the grooves and reduction of the total thickness of the billet to that desired for the narrow strips wherewith the dimension of the residues of said weld-preventing material in the direction of the thickness of the strips is reduced coordinately with the reduction of such total thickness, and then applying forces to the rolled product whereby to over-stress and effect separation along the lines of said residues of the weld-preventing material applied to the groove walls and thereby separate the rolled product into a plurality of narrow strips.

2. The method as in claim 1, in which the longitudinal grooves are provided at opposed surfaces of the billet, with said grooves aligned in pairs, whereby the rolled product has the residues of the weld-preventing material of said pairs of grooves aligned and constituting parallel longitudinal regions of weakness in said rolled product.

3. The method as in claim 2, in which the rolled product is subjected to repeated flexings in opposite directions to effect the separation.

4. The method of preparing narrow strips of material each having an internal discontinuity between surface laminations, the laminations being connected at the lateral edges of the discontinuity, which comprises preparing a billet of the material with a plurality of internal longitudinal channels spaced laterally from one another and from the longitudinal edges of the billet by portions of solid metal extending from face to face of the billet, said channels containing extensible weld-preventing material, said billet having a plurality of longitudinal external grooves at a roll-engaging face thereof, each of said grooves being located opposite one of the said solid metal portions, the parts of said solid metal portions beneath the roots of said grooves being effective to maintain integrity of the billet from side to side during rolling, said grooves being spaced differentially across said roll-engaging face so that two adjacent grooves near an edge are at a different spacing than two adjacent grooves near the center of width, placing a weld-preventing material on a wall of each groove, rolling the billet whereby to cause lateral closure of the grooves and reduction of the total thickness of the billet wherewith lateral spreading of points spaced across the width occurs during rolling, terminating the rolling when the lateral spreading has brought the residues of the grooves to predetermined spacing thereof, and applying forces to the rolled product whereby to over-stress and effect separation along the lines of the groove residues.

5. The method as in claim 4, in which a wall of each

groove receives a coating of weld-resisting material prior to rolling.

6. The method as in claim 4, in which two opposed surfaces of the billet have longitudinal external grooves of V shape, arranged in pairs with the points of the V's located in a surface at right angles to said opposed surfaces.

7. The method as in claim 4, in which the grooves have V cross-sections, said cross-sections of the grooves are tilted relative to one another, with the grooves adjacent the lateral edges of the billet having a greater tilt than grooves nearer to the center of the width thereof.

8. The method of preparing narrow strips of metal each having an internal discontinuity between surface laminations, said laminations being integrally connected at the edges of each strip, which comprises preparing a billet having internal longitudinal cores of extensible weld-preventing material, said cores being alined transversely of the billet and separated by metal spacers integral with the surface metal of the billet, said billet also having external grooves in roll-contacting surfaces of the billet and alined with the said metal spacers, the metal of said spacers beneath the roots of the grooves being effective to maintain integrity of the billet from side to side during rolling, each groove having a coating of weld-preventing material on a wall thereof, rolling the billet whereby to reduce its thickness to that desired for the strips wherewith the grooves are closed by lateral spreading of adjacent billet material to provide smooth surfaces and with the residues of said coating extending inward from the respective surface, and applying forces to the rolled product whereby to over-stress and effect separation into narrow strips along the lines of the groove residues, each strip having an internal discontinuity from the residue of a said core.

9. The method as in claim 8, in which grooves are provided in opposed surfaces of the billet, the grooves being alined in pairs along geometric surfaces intersecting said opposed surfaces and each passing through a said spacer.

10. The method as in claim 8, in which the grooves are of V cross-section, and the cross-sections of the grooves are relatively tilted, the tilt being progressively greater from the center of width toward the edges.

11. The method as in claim 10, in which the grooves are provided at the opposed surfaces of the billet, and arranged in pairs, with the points of the V's of each pair lying in a geometric surface normal to said opposed surfaces and passing through a said spacer.

12. The method as in claim 8, in which a pair of alined grooves are provided between an edge of the billet and the edge of the adjacent core, whereby to provide in the rolled product a longitudinal weakening parallel to the edge of the residue of said core along which may be severed a strip at a predetermined distance from the residue of said core.

13. The method of preparing a strip having a plurality of internal longitudinal discontinuities spaced across its width and with longitudinal weakenings in planes intersecting the body material between the discontinuities, which comprises preparig a billet having a like number of longitudinal discontinuities therein and with billet metal extending as spacing regions between each two of said discontinuities, said discontinuities containing extensible weld-preventing material, and including the forming on an external roll-contacting surface of the billet of longitudinal grooves spaced at unequal intervals across the width of the billet, the metal beneath the roots of the grooves being effective to maintain integrity of the billet from side to side during rolling, the spacing being greater toward the side edges than near the center, providing anti-welding material in the grooves, and rolling the billet so that the thickness is reduced to that of the desired strip

wherewith the anti-welding material extends longitudinally in proportion to the decrease in billet thickness and therewith causes the strip to have a laminated structure at the said discontinuities, wherewith the said grooves become closed during the rolling and the anti-welding material therein provides longitudinal weakenings along the strip, and wherewith the lateral spreading of the billet during rolling causes the weakenings to be presented at uniform intervals across the width of the strip and each opposite the rolled residue of a said metal spacing region.

14. The method of preparing narrow sections of metal each having an internal discontinuity between surface laminations, said laminations being integrally connected at the edges of each section, which comprises preparing a billet having internal cores of weld-preventing material extending along its length, said cores being alined transversely of the billet and separated by metal spacers integral with the surface metal of the billet, said billet also having external grooves in roll-contacting surfaces of the billet and alined with the said metal spacers, the metal beneath the roots of the grooves being effective to maintain integrity of the billet from side to side during rolling, rolling the billet whereby to extend its length and reduce its thickness to that desired for the sections wherewith the external grooves are closed by lateral spreading of adjacent billet metal to provide smooth surfaces, and applying forces to the rolled product at laterally spaced regions thereof whereby to over-stress and effect separation into narrow sections along the lines of the groove residues, each section having an internal discontinuity from the residue of a said core.

15. An article of manufacture which is a billet of rollable metal and having metal surface portions separated in longitudinally extending regions of the billet by a longitudinal internal channel at each such region and having integrating longitudinally extending metal spacer portions between each two adjacent regions, and a plurality of external longitudinal grooves in a roll-contacting surface of the billet, each said groove being spaced laterally relative to and between the lateral edges of two adjacent internal channels and extending into the respective metal spacer portions, with a wall of each groove having a coating of weld-preventing material.

16. An article of manufacture which is a billet of rollable metal and having metal surface portions separated in longitudinally extending regions of the billet by a longitudinal internal channel at each such region and having integrating longitudinally extending metal spacer portions between each two adjacent regions, and a plurality of pairs of external longitudinal grooves in the roll-contacting surfaces of the billet, each pair of said grooves being spaced laterally relative to and between the lateral edges of two adjacent internal channels and extending into the respective metal spacer portions, with a wall of each groove having a coating of weld-preventing material, each said groove being of V-shape and having the bisectors of the angles between the groove walls located at acute angles to the said opposed surfaces.

#### References Cited in the file of this patent

#### UNITED STATES PATENTS

|           |           |                |
|-----------|-----------|----------------|
| 140,762   | Bolton    | July 15, 1873  |
| 1,209,949 | Dodds     | Dec. 26, 1916  |
| 1,926,320 | Trembour  | Sept. 12, 1933 |
| 2,079,213 | Ingersoll | May 4, 1937    |
| 2,215,933 | Offutt    | Sept. 24, 1940 |
| 2,375,334 | Valyi     | May 8, 1945    |
| 2,377,857 | Belanger  | June 12, 1945  |
| 2,423,810 | Goulding  | July 8, 1947   |
| 2,766,514 | Adams     | Oct. 16, 1956  |
| 2,851,770 | Fromson   | Sept. 16, 1958 |
| 2,986,810 | Brick     | June 6, 1961   |